

## UNITED STATES PATENT OFFICE

2,537,513

## PRINTING INK

Joseph G. Curado, Bergen County, N. J., assignor  
to Sun Chemical Corporation, New York, N. Y.,  
a corporation of Delaware

No Drawing. Application April 30, 1947,  
Serial No. 745,105

4 Claims. (Cl. 106—31)

1

This invention relates to printing inks and to vehicle components of such inks.

One object of the present invention is to provide an ink material of such characteristics that proper printing, without fill-in from half tone printing plates can be secured, and which has the further characteristics of setting as an imprinted film to substantially non-offsetting, non-smudging conditions upon the application of moisture thereto.

Another object of the present invention is to provide an ink material having the characteristics of printing without fill-in and of setting as above described, and in which a major proportion of the binder material is a modified beta-naphthol pitch.

Another object of the present invention is to provide a process for modifying beta-naphthol pitch to secure a binder ingredient for ink materials which give satisfactory printing from half tone plates without fill-in.

Other objects of the present invention will be apparent from the following description and appended claims.

Moisture setting inks, in which the vehicle component contains a water-immiscible binder material dissolved or dispersed in a water-miscible carrier component, have been successfully used in many fields of printing. For example, books, magazines, newspapers and the fields of carton and label printing wherein ink materials are desired which have characteristics of extremely rapid setting to non-offsetting, non-smudging films and which provide imprinted films which are substantially odorless. In such type of printing, the printing operation ordinarily is effected from line cuts or plates, and almost all of the printing is concerned with the reproduction upon the base material of a solid print.

Some difficulties have been encountered in utilizing such inks as have hitherto been available in the field of publication printing, for example, books, magazines, newspapers and the like. In such printing operations a considerable proportion of the printing is effected from half tone plates, and to secure satisfactory printing, substantially faithful reproduction of the half tone dots is required without fill-in of the intervening spaces of the non-printed surface with ink material. When such fill-in occurs, the effectiveness of the half tone printing is objectionably altered in that the reproduction on the imprinted surface contains ink in portions not intended to be printed. The result is a poor print.

2

By the present invention there is provided an ink material which is of such characteristics that successful printing from half tone plates without objectionable fill-in can be secured and which retains the desirable characteristics of setting, as an imprinted film, to non-offsetting, non-smudging conditions upon the application of moisture. Such ink material contains as a major proportion of the binder constituent a modified material secured from beta-naphthol pitch.

Beta-naphthol pitches are still bottoms obtained in the production of beta-naphthol, when the pure product is distilled from the crude mixture obtained by the fusion of naphthol sulfonic acid with alkali hydroxide, followed by separation of the crude from the reaction mixture. In United States Patents Nos. 2,415,827 and 2,415,828, issued on February 18, 1947, in the name of Ernest D. Lee and assigned to Interchemical Corporation, there are described ink materials in which beta-naphthol pitch is utilized as a binder constituent. I have found that inks such as those described in the above patents are not satisfactory in publication printing or in other printing in which half tone printing plates are used. However, it has been found, according to the present invention, that by proper modification of such pitch materials, inks can be prepared which are completely satisfactory for such printing from half tone surfaces without objectionable fill-in.

I have found that beta-naphthol pitches generally contain a relatively minor proportion of glycol-insoluble constituents. The amount of such constituents generally is within the range of 0.1 to 2 per cent by weight of the beta-naphthol pitch. Further, I have found that the presence of this relatively minor amount of glycol-insoluble constituent is critically responsible for the failure of such beta-naphthol pitches, unmodified, to print properly from half tone printing plates without objectionable fill-in. As a result of my research, I believe that the reason why such unmodified beta-naphthol pitches are unsatisfactory is that, upon dissolving or dispersing in a water-miscible liquid carrier component of the type utilized in moisture setting inks, this relatively minor proportion of glycol-insoluble constituent does not properly disperse or dissolve in the liquid carrier component. While vehicles prepared, containing such glycol-insoluble constituents, appear to be homogeneous, upon printing with inks prepared containing such vehicle components, I have found that unsatisfactory

printing from half tone plates is secured, in that objectionable fill-in upon printing is obtained.

In accordance with the present invention I have found that when a vehicle is prepared in which the binder constituent, or a major proportion thereof, is a modified beta-naphthol pitch, that satisfactory printing from half tone plates without fill-in is secured. One satisfactory method of securing such modified beta-naphthol pitch consists in treating this material with a 5 solvent as dipropylene glycol under conditions such that solution of glycol-soluble ingredients is secured. After solution is secured of those portions of the beta-naphthol pitch which are soluble, the mixture then is treated, satisfactorily by filtration, to separate from the solution, that portion of the beta-naphthol pitch which is insoluble in the glycol. Upon such treatment I have found that the modified beta-naphthol 15 pitch furnishes a satisfactory binder material for moisture setting inks characterized by the printing qualities outlined above and by its ability, when used in such inks, to furnish a non-offsetting, non-smudging film containing pigment, upon the application of moisture to the imprinted 20 film.

In preparing the ink materials, the glycol solution of modified beta-naphthol pitch, prepared as hereinafter described, may be modified, if necessary, by the addition of additional water-miscible liquid carrier component to provide an 25 ink vehicle of satisfactory viscosity, and coloring materials such as pigments and toners dispersed therein to give an ink of the superior characteristics of the present invention.

Liquid carrier components satisfactory for use in preparing ink material of the present invention include water-miscible materials in which the modified beta-naphthol pitch can be dissolved or dispersed. Examples are glycols, such as 30 ethylene glycol, propylene glycol, 2-methyl-2,4-pentanediol and the like, glycol ethers such as the ethyl ether of ethylene glycol, butyl ether of ethylene glycol and the like, esters of glycol ethers such as the acetic acid ester of the ethyl ether of ethylene glycol, polyglycols such as diethylene 35 glycol and dipropylene glycol, polyglycol ethers such as the ethyl ether of diethylene glycol and butyl ether of diethylene glycol, esters of polyglycol ethers such as the acetic acid ester of the butyl ether of diethylene glycol, and mixtures of 40 these materials.

Illustrative of one satisfactory method of effecting preparation of a modified beta-naphthol pitch is the following example.

#### Example 1

Forty pounds of beta-naphthol pitch are 45 mixed with sixty pounds of dipropylene glycol and the mixture warmed under agitation conditions, to effect solution of the soluble material present, which in the case of quantities above described, may satisfactorily be accomplished by stirring the admixture at 100° C. for one hour. Upon completion of this step, the mixture secured then is 50 filtered. Satisfactorily, the filtration operation can be effected by adding to the warmed mixture 5 pounds of a diatomaceous silica filter aid and one pound of fuller's earth, and thereafter filtering the admixture in a high pressure compression filter having a circular filter membrane 71 inches in diameter. The filtrate from such operation 55 comprises a satisfactory ink material of the present invention.

Illustrative of an ink material satisfactory for commercial printing containing the above vehicle is the following.

#### Example 2

|                           | Pounds |
|---------------------------|--------|
| Carbon Black.....         | 10     |
| Vehicle of Example 1..... | 72     |
| Dipropylene glycol.....   | 18     |
|                           | 100    |

This ink has satisfactory working properties for printing on letter press equipment. Upon printing from half tone printing plates, the ink printed with substantially no fill-in and gave excellent reproduction of the printing surface.

An ink prepared containing the same proportions of ingredients, but in which an unmodified beta-naphthol pitch such as that described in the Lee Patents Nos. 2,415,827 and 2,415,828 was employed, when printed under the same conditions, showed a substantial fill-in in half tone printing with consequent failure to reproduce faithfully the printing surface and gave a print in which the reproduction did not seem to be clean and sharp.

Other pigment materials may be used in place of the carbon black. Also, with carbon black, toning pigments may be employed to give slightly different effects, the toners normally making black print look slightly darker than when carbon black is used alone.

The modified beta-naphthol pitch also may be employed in conjunction with other binder materials which have satisfactory characteristics for utilization in inks adapted for moisture setting after the printing. Examples of such binder materials are rosin modified by reaction with maleic anhydride, terpenes modified by reaction with maleic anhydride, zein, shellac and analogous binder materials which are soluble or dispersible in the liquid component and insoluble in water.

In the illustrative Example 1, the quantities of diatomaceous silica filter aid and fuller's earth utilized are satisfactory under the particular filtration conditions set forth. With other quantities of materials and different size filters, other quantities of such materials naturally will be employed to obtain satisfactory filtration operations. It appears to be desirable to have present during such filtration an amount of such filter aid and fuller's earth sufficient to form a layer approximately one inch thick on the filter membrane, using the particular filtering system described by way of illustration.

The effectiveness of the illustrative filtration method may be explained on the basis of the nature of the glycol-insoluble constituents normally present in unmodified beta-naphthol pitch. Upon treatment with dipropylene glycol as above set forth, such insoluble constituents form swelled, gelatinous aggregates which quickly plug up ordinary filter membranes and reduce the effectiveness of the filtration operation. Upon addition of the filter aid and fuller's earth, a bed of material is formed which increases the effectiveness of filtration and prevents formation of a film of gelatinous particles of glycol-insoluble constituents on the filter membrane.

With other methods of filtration, such filter aids may not be necessary. What is important is the securing of the removal of such glycol-insoluble constituents from the beta-naphthol pitch 75 to secure a binder material, which, when utilized

in printing inks of the character described, has the superior characteristics upon printing hereinbefore set forth.

Other liquid materials may be utilized in the modification procedure in place of dipropylene glycol. Such materials include the liquid carrier components above described, that is, the water miscible glycols, glycol ethers, esters of glycol ethers, polyglycols, polyglycol ethers and esters of polyglycol ethers. As a matter of economy, it generally has been found satisfactory to utilize, in the modification procedure, the material which is to be employed as the major liquid carrier component of the final ink material, since it appears that the glycol-insoluble constituents of unmodified beta-naphthol pitch are likewise insoluble in such other liquid carrier components.

While the above described examples constitute preferred embodiments of the invention, changes may be made therein without departing from the scope of the invention as defined in the appended claims.

What is claimed is:

1. An ink material having the properties of printing without fill-in from half tone printing plates and of setting as an imprinted film, to substantially non-offsetting, non-smudging conditions upon the application of moisture thereto, and comprising a binder component and a liquid carrier component, said binder component being beta-naphthol pitch having less than 0.1 per cent by weight of glycol-insoluble constituents, and the liquid carrier component being 2-methyl-2,4-pentanediol.

2. An ink material having the properties of printing without fill-in from half-tone printing plates and of setting as an imprinted film, to substantially non-offsetting, non-smudging conditions upon the application of moisture thereto, and comprising a binder component and a liquid carrier component, said binder component being the glycol-soluble extract from beta-naphthol pitch, and the liquid carrier component being 2-methyl-2,4-pentanediol.

3. An ink material having the properties of printing without fill-in from half-tone printing plates and of setting as an imprinted film, to substantially non-offsetting, non-smudging conditions upon the application of moisture thereto, and comprising a coloring material dispersed in a vehicle component, said vehicle comprising a binder component and a liquid carrier component, said binder component being beta-naphthol pitch having less than 0.1 per cent by weight of glycol-insoluble constituents, and the liquid carrier component being 2-methyl-2,4-pentanediol.

4. An ink material having the properties of printing without fill-in from half-tone printing plates and of setting as an imprinted film, to substantially non-offsetting, non-smudging conditions upon the application of moisture thereto, and comprising a coloring material dispersed in a vehicle component, said vehicle comprising a binder component and a liquid carrier component, said binder component being the glycol soluble extract from beta-naphthol pitch, and the liquid carrier component being 2-methyl-2,4-pentanediol.

JOSEPH G. CURADO.

#### REFERENCES CITED

The following references are of record in the file of this patent:

#### UNITED STATES PATENTS

| Number       | Name        | Date           |
|--------------|-------------|----------------|
| 2,002,652    | Alexandroff | May 28, 1935   |
| 2,139,242    | Mocls       | Dec. 6, 1938   |
| 2,289,638    | Erickson    | July 14, 1942  |
| 2,323,710    | Erickson    | July 6, 1943   |
| 2,415,827    | Lee         | Feb. 18, 1947  |
| 2,415,828    | Lee         | Feb. 18, 1947  |
| 40 2,449,230 | Irion       | Sept. 14, 1948 |

#### OTHER REFERENCES

Grempe: "Farber Zeitung," 26, (1915), pages 322 and 323.